

## UNITED STATES PATENT OFFICE

LATIMER D. MYERS AND LOU A. STEGEMEYER, OF CINCINNATI, OHIO, ASSIGNOR TO THE TWITCHELL PROCESS COMPANY, OF CINCINNATI, OHIO, A CORPORATION OF OHIO

## PROCESS OF DEGUMMING SILK

No Drawing.

Application filed March 16, 1929. Serial No. 347,729.

This invention relates to a process of treating raw silk to remove from it the natural gum. Genuine silk is produced by the silk-worm (*Bombyx mori*), and comprises the fiber which is known as fibroin, and the yellow gum sericin which is about 20 to 30% of the weight of the silk fiber.

This sericin coats the silk fibers and imparts to the silk a harsh, stiff feeling and also interferes very materially with the dyeing of the silk. It is therefore necessary to remove the sericin from the silk, which process is usually called degumming, discharging or stripping.

15 It is generally preferred to practice this process after the silk has been woven into cloth or fabric, though it may be carried on if desired beforehand. The removal of the sericin presents quite a problem because it is only slightly soluble even in hot water, and agitation, boiling or rubbing are very undesirable because of their physical effect upon the silk itself.

In carrying on the process previously practiced, 350 pounds of silk are suspended in a bath made up from 2500 gal. of soft water and 250 lbs. of olive oil, red oil or other low titer soap. The temperature of the bath is held just below the boiling point, say 205° F. After two hours, the silk is removed from the first bath and treated for approximately twenty minutes in a second bath containing 2500 gal. of water and 50 lbs. of soap. The original degumming bath may be used to degum two additional 350 lb. batches of silk by adding seventy-five lbs. of soap before each boil. After three boils the bath becomes heavily charged with sericin and is either discarded or used in the dye house under the name of boiled liquor.

There are many disadvantages of this process, however, the first of which is the high consumption of relatively expensive fatty acid soap. Second, the time of the treatment is excessive and the amount of heat required for the long treatment is an undesirable economic factor. Third, a scum is left on the surface of the bath and adheres to the silk as it is withdrawn, and if not completely removed by a second bath, causes

irregularities in later dye operations. Fourth, it is difficult to wash all of the fatty acid soap from the silk without injuring it physically, and the portions or traces of the fatty acid soap left in the silk are decomposed in the acid dye bath to fatty acids which are insoluble and cause uneven dyeing of the fabric.

The object of this invention, therefore, is to provide a process of degumming silk which is free from the disadvantages outlined in the previous paragraph.

Another object of this invention is to provide a material or reagent adapted to wash or remove the sericin from silk.

This invention comprises treating the natural silk alone or associated with other fibers or materials with an aqueous alkaline solution and an aqueous solution of a powerful emulsifying agent which removes the natural gum and also any oil or other similar material which may have been deposited upon the fibers during some previous treatment. This emulsifying agent is so powerful that it prevents the formation of any scum upon the surface of the bath in which the silk fiber is treated. It is likewise the concept of the inventors to use an emulsifying agent which is soluble in acid dye baths of the sort in which the silk is to be later treated so that no unevenness of dyeing will result from traces of the emulsifier remaining upon the silk fiber.

The alkaline solution renders the sericin soluble somewhat in proportion to its alkalinity, so research has been undertaken to establish what alkalinity can be used with safety in the presence of the preferred emulsifying agent of this invention.

This preferred reagent comprises mineral oil sulphonates, recovered as by-products in the practice of the Petroff-Humphrey process of refining mineral oil such as lubricating stock into white oil and the light colored technical oils. This process is exemplified by the following patents:

Petroff 1,087,888 February 19, 1914  
Humphrey 1,286,179 November 26, 1918

Mineral oil sulphonates fall in two general classes. The mahogany sulphonates or oil

layer sulphonates recovered and extracted from the oil layer in the refining operation, and the sludge sulphonates recovered from the sludge layer formed in the refining operation. We prefer to use the mahogany sulphonates for degumming silk because they are more powerful as emulsifiers than the sludge layer sulphonates, and also because they have less tendency to discolor the silk. 10 These sulphonates are most available in the form of sodium salts, though other water soluble salts may be used.

Our investigation has determined that in the presence of the mahogany sulphonate it 15 is possible to carry the alkali content of the degumming solution to as high as .03% sodium hydroxide without injuring the silk fiber. The general range of alkalinity recommended is, therefore, between .01 and .03% 20 sodium hydroxide solutions. Other alkalies or potential alkalies may be used instead of the sodium hydroxide, the quantities being adjusted to provide equivalent alkalinity.

The amount of mahogany sulphonates used 25 is less critical but the use of a .5 to 1% aqueous solution (based on weights) is recommended. The silk is preferably immersed in this aqueous solution containing .03% sodium hydroxide and .5 to 1% mahogany sulphonate at a temperature slightly below boiling for a period of between 10 and 45 minutes. 30 The surface of the degumming bath is entirely free from scum due to the unusual emulsifying powers of the mahogany sulphonate. 35 One bath, with replacement of the alkali which has been used up in previous treatment, may be used for at least four batches of silk before the concentration of sericin becomes harmfully high. This result is possible 40 because of the unusual colloidal power of the mahogany sulphonates to disperse the sericin which has been saponified by the alkali. Since the alkali is used up by each treatment, the degummed silk fiber is not injured by the 45 solution.

Before being placed in the dye bath the silk is rinsed in water but should any of the mahogany sulphonate remain on the silk no harm is done since the acid dye bath converts 50 the mahogany soap to mahogany acid which is also readily soluble. The silk so degummed, therefore, dyes evenly, first, because it has not been contaminated with any scum, and secondly, because traces of the emulsifier 55 are soluble in the dye bath.

For example, a bath is made up as follows:

10,000 parts = 1200 gal. H<sub>2</sub>O

100 parts = 100 lbs. Na mahogany sulphonates

3 parts = 4 lbs. NaOH

These quantities provide a process wherein the sericin is saponified and completely removed from the silk fiber and the alkali content of the treatment bath simultaneously

substantially exhausted so that after the silk fiber is exposed, the solution is not of sufficient strength to be injurious to it. This bath will degum 150 lbs. of silk fabric within thirty minutes and without injury to the silk. 70

From this example it will be observed that the preferred reagent comprises substantially 100 parts mahogany sulphonates to 3 parts sodium hydroxide by weight. 75

A substantial problem resides, however, in constituting an entirely homogeneous reagent of mahogany sulphonates and alkali, that is, a reagent in which the alkali will not settle or separate from the sulphonates, so that some portion of the particular batch contains a greater percentage of alkali than some other portion. Moreover, the mahogany sulphonates alone are quite viscous and gummy and consequently hard to pour, handle, 80 and measure with accuracy. 85

If water is added in an effort to thin down the material the alkali salts out the mahogany sulphonates or a portion of the mahogany sulphonates. If, however, a water soluble solvent, such as methyl alcohol, is added to the mahogany sulphonates and alkali an entirely homogeneous body is formed in which the components do not salt out or separate. For instance, a satisfactory reagent is 95 constituted as follows:

3 parts sodium hydroxide  
110 parts sodium mahogany sulphonates  
containing 10% water  
8 parts 95% methyl alcohol. 100

If desired, oil may be added to this mixture to further reduce the viscosity and to increase the solubility of the substance without causing a separation of the alkali. Otherwise expressed, we add to the mahogany sulphonates and alkali a mutual solvent for the alkali and sulphonates such as an aqueous alcohol or the like, and this effects a homogeneous admixture of the mahogany sulphonates and alkali, so that all portions of a given batch contain substantially the same percentage of components. 110

Having described our invention, we desire to be limited only by the ensuing claims: 115

1. A material adapted to degum silk, said material comprising mineral oil sulphonates, an alkali, and a liquid in which the sulphonates and alkali are both soluble.

2. A material adapted to degum silk, said material comprising, mineral oil sulphonates, an alkali, and alcohol. 120

3. A homogeneous material adapted to degum silk, said material comprising substantially 110 parts mahogany sulphonates containing about 10% water, 3 parts sodium hydroxide, and 8 parts 95% methyl alcohol. 125

4. The art of effecting a substantially complete removal of sericin from silk without injury to the silk, said art comprising, subject- 130

- ing the silk bearing the sericin simultaneously to the chemical and colloidal action of a hot aqueous solution, the chemical action being provided by an alkali in said solution 5 equal in strength to between .01 and .03% sodium hydroxide, the colloidal action being provided by water soluble salts of mahogany sulphonic acids adapted to disperse the sericin saponified by the alkali throughout the 10 solution without scum formation.
5. The art of effecting a substantially complete removal of sericin from silk without injury to the silk, said art comprising, subjecting the silk bearing the sericin simultaneously to the chemical and colloidal action of a hot aqueous solution, the chemical action being provided by an alkali in said solution equal in strength to between .01 and .03% sodium hydroxide, the colloidal action 15 being provided by water soluble salts of mahogany sulphonic acids adapted to disperse the sericin saponified by the alkali throughout the solution without scum formation, the quantity of the treating solution being so adjusted to the quantity of silk treated that the 20 available alkali content of the solution is substantially reduced by the saponification of the sericin on the silk so that the treating solution is not injurious to the silk fiber as it 25 becomes exposed by removal of the sericin.
6. The method of degumming successive batches of silk in a single treating bath, said method, comprising, alkalinizing the treatment bath before each batch of silk is introduced, the quantity of alkali introduced being 30 related to the quantity of sericin to be saponified by its action so that the available alkali in the bath is substantially reduced by its action on the sericin, maintaining the removed 35 sericin in a dispersed condition throughout the bath without scum formation by virtue of the presence in the treating bath of water soluble salts of mahogany sulphonic acids, and replacing alkali after each bath in relation to the next succeeding batch of silk 40 to be degummed.
7. The art of effecting a substantially complete removal of sericin from silk without injury to the silk, said art comprising, subjecting the silk bearing the sericin simultaneously to chemical and colloidal action of a hot aqueous solution, chemical action being provided by an alkali adapted to saponify the 45 sericin present on the silk being treated, colloidal action being provided by water soluble salts of mahogany sulphonic acids adapted to emulsify the saponified sericin.
8. The art of effecting a substantially complete removal of sericin from silk without injury to the silk, said art comprising, subjecting the silk bearing the sericin simultaneously to a chemical action and a colloidal action in a hot aqueous solution, the chemical action being provided by an alkali and the colloidal 55 action by water soluble salts of mahogany 50 55 60 65 70 75 80 85 90 95 100 105 110 115 120 125 130
- sulphonic acids, the process being carried out with quantities of materials bearing substantially the following relationship to one another as to quantities:—150 pounds of raw silk, 1200 gallons water, 4 pounds sodium hydroxide, 100 pounds of sodium mahogany sulphonates.
- In witness whereof, we hereunto subscribe our names.
- LATIMER D. MYERS. 75  
LOU A. STEGEMEYER.